# EUROPEAN PATENT SPECIFICATION

(11) **EP 3 225 321 B1**
(45) Date of publication and mention of the grant of the patent: **30.08.2023**
(21) Application number: 15863977.3
(22) Date of filing: 12.11.2015
(51) Int. Cl.: B21D 5/01

(54) **A METHOD OF PRODUCING A STEEL PIPE**
VERFAHREN ZUR HERSTELLUNG EINES STAHLROHRS
PROCÉDÉ DE FABRICATION D'UN TUYAU EN ACIER

(30) Priority: 25.11.2014 JP 2014237608
(43) Date of publication of application: 04.10.2017
(73) Proprietor: JFE Steel Corporation, Tokyo 100-0011 (JP)
(72) Inventor: HORIE, Masayuki, Tokyo 100-0011 (JP); TAMURA, Yukuya, Tokyo 100-0011 (JP); MIWA, Toshihiro, Tokyo 100-0011 (JP); TATENO, Junichi, Tokyo 100-0011 (JP)
(74) Representative: Grünecker Patent- und Rechtsanwälte PartG mbB
(86) International application number: PCT/JP2015/081818
(87) International publication number: WO 2016/084607

(56) References cited:
- JP-A- S53 112 260
- JP-A- S53 112 260
- JP-A- S55 139 117
- JP-A- S60 130 419
- JP-A- 2012 250 285
- JP-A- 2012 250 285
- US-A- 1 387 199
- US-A- 2 479 336
- US-A- 4 149 399

## Description

### TECHNICAL FIELD

The present invention relates to a method for producing a steel pipe according to the preamble of claim 1. Such a method is known from JP 2012 250 285 A. The present invention relates in particular to a method suitable for producing a thick and large-diameter steel pipe used for a line pipe or the like.

### BACKGROUND ART

As a technique for producing a thick and large-diameter steel pipe used for a line pipe or the like, a so-called UOE forming technique is widely used which presses a steel plate having a predetermined length, width and plate thickness into a U-shape, press-forms the steel plate into an O-shape to make an open pipe, thereafter its gap portion is butt-jointed by welding, and enlarges its diameter (so-called pipe expansion) to further improve the roundness.

In the above-described UOE forming technique, however, since there is a need for a high pressing force in the process of pressing the steel plate to form the steel plate into a U-shape and an O-shape, it cannot help using a large-scale press machine.

Therefore, recently, a technique for decreasing the pressing force has been considered upon producing this kind of steel pipe.

As a prior art related to this point, Patent Document 1 discloses a method of preliminarily forming a material in a C-shape forming process and a U-shape forming process, then performing an O-shape forming process thereon, so that a deformation mode of the material to be formed becomes fitting to dies at both top and bottom portion in the O-shape forming process. Further, Patent Document 2 discloses a method of changing a position of a butted part of a U-shaped steel plate to dies by performing a plurality of O-shape presses on the U-shaped steel plate and also rotating the U-shaped steel plate during the O-shape press, and Patent Document 3 discloses a method of performing the O-shape press on a member formed into a U-shape by a U-shape press with an insert liner which is applied for larger outer diameter pipe to an intermediate outer diameter.

As other prior arts, Patent Document 4 discloses a forming method in which a strain detector capable of detecting the inclination or distortion of a bending member mounted on a slide is disposed, the bending member is disposed in a tiltable or parallel-movable manner corresponding to the detection of the inclination or distortion by the strain detector, and the bending member is inclined or parallel moved to be subjected to press-forming so that an amount of distortion is smaller than an amount of inclination or an amount of distortion of the bending member when press-forming a material to be formed into a pipe shape. Patent Document 5 discloses a method of forming a slit pipe equipped with a non-circular preform by performing the slight forming compared to other bending steps in at least one bending step of acting on the inner surface of the plate material on left and right with respect to a center defined by a longitudinal axis of an upper tool that enters a plate material to be progressively formed, and thereafter, forming a finished slit pipe by appropriately applying a pressing force acting on an area formed slightly in advance on both sides of the center from the outside to the non-circular preform. Furthermore, Patent Document 6 discloses a method of forming a pipe with a closed slit portion, by applying the plastic deformation only to the flat portion of at least one location in the preformed body having a flat portion between at least two bent portions bent to a predetermined pipe curvature.

### PRIOR ART DOCUMENTS

### PATENT DOCUMENTS

Patent Document 1: JP-A-S55-139117
Patent Document 2: JP-A-H1 1-285729
Patent Document 3: JP-A-2002-178025
Patent Document 4: JP-A-2005-21907
Patent Document 5: JP-A-2012-250285
Patent Document 6: US Patent No. 4,149,399

### SUMMARY OF THE INVENTION

### TASK TO BE SOLVED BY THE INVENTION

Meanwhile, the conventional press-forming techniques have problems as described below, and hence there is still room for improvement.

That is, in Patent Documents I to 3, a circumferential length on a forming surface of the die is set to be substantially equal to the width size of a plate material (a raw plate), and the plate material is formed into a pipe shape by bringing a extending portion of the material into contact with a forming surface of the die during deformation of the O-shape press to adjust it into a shape of the forming surface of the die. However, when a contact portion with the die is increased, the pressing force is gradually increased, and there is a need for a large press machine.

In a technique particularly aimed at a thick and high-strength material, a large pressing force is needed and thus the material is not completely pressed in the O-shape press, whereby a degradation of the shape cannot be avoided.

Meanwhile, according to the methods described in Patent Documents 4, 5 and 6, although they do not accompany an increase in pressing force as in Patent Documents 1 to 3, since the material to be formed or the non-circular preform is separately formed on each of left and right sides, when the amount of deformation differs on the left and right sides, there is a risk of formation of a step difference (offset) in the gap portion or the slit portion serving as a welded portion. Further, in these methods, the deformation is locally concentrated when trying to deform a shape to a desired shape at one time, and there is a fear of worsening the roundness. Accordingly, deformations of several times are inevitable, and there is also a limit in efficient production.

The present invention is to provide a producing method of efficiently producing a steel pipe having high roundness without requiring an excessive bending force (load).

### SOLUTION FOR TASK

The present invention proposes as a solution a method of producing a steel pipe with the features of claim 1; i.e. subjecting a plate material which is bent at width end portion to at least one bending along its widthwise direction to provide a preformed body having a U-shaped cross-section, pressing the preformed body by applying a bending force to thereby form an open pipe with a gap portion in its longitudinal direction, and butt-joining end surfaces of the gap portion of the open pipe to each other, wherein a lightly-bent portion to which a slighter curvature is applied as compared to other regions or a non-bent portion in which the bending is omitted is provided in at least a part of the plate material in a process performing the bending on the plate material, and a bending-force is applied to a part spaced apart from the center of the lightly-bent portion or the non-bent portion by a distance within a range of W/4 ± 0.07W in a width end portion direction of the plate material, where W is the width of the plate material, without constraining the lightly-bent portion or the non-bent portion in a process pressing the preformed body into the open pipe, wherein the length of the lightly-bent portion or the non-bent portion along the widthwise direction of the plate material is not more than 10% of the plate material width.
Here, the open pipe refers to a pipe body of a state in which the plate material is formed into a cylindrical shape and a gap portion is formed between plate end portions facing each other.

Preferred embodiments of the inventive method are defined in the appended dependent claims.
Preferably, a pressing die with a pair of bending tools is used, wherein at least one of the bending tools has a circular arc surface having a width center that lies on an axis of symmetry of the press die, and a forming surface having an inclined surface which leads to each of both ends of the circular arc surface and is directed toward the forming center of the press die. Further, the circular arc surface preferably has a central angle of not less than 28°, an angle formed between the inclined surface and a straight line intersecting with a straight line passing through a widthwise center of the circular arc forming surface is preferably not less than 14°, and a surface having a radius of not more than 1.2 times the diameter of a steel pipe to be produced may be applied as the circular arc surface.

### EFFECTS OF THE INVENTION

According to the method of producing a steel pipe of the present invention, , it is possible to efficiently form a steel pipe having high roundness with a relatively small bending force.

Further when the lightly-bent portion or the non-bent portion is provided at a part spaced apart from a width end portion of the plate material by amount of W/4, and the preformed body having a U-shaped cross-section is pressed into an open pipe, the part is not restricted by the press die, and thus, it is possible to suppress an increase in forming reaction force.

According to the method of producing a steel pipe of the present invention, since a length of the lightly-bent portion or the non-bent portion along the widthwise direction of the plate material is not more than 10% of the plate width dimension, it is possible to obtain an open pipe having a small open amount of the butted portion, while maintaining the dimensional accuracy.

At the time of pressing of the preformed body by applying a bending force thereto, the preformed body is preferably supported at a part at least away from an extension line on which the bending force acts, and the pressing of the preformed body is started under the condition of θf > θs in which an opening angle of the preformed body defined based on the part supporting the preformed body is defined by θs, and an angle of the bending force is defined by θf, so that the lightly-bent portion or the non-bent portion is deformed so as to extend outward.

At the time of pressing of the preformed body, a press die provided with a forming surface not coming into contact with the lightly-bent portion or the non-bent portion is preferably used, such that it is possible to press the preformed body while decreasing the bending force.

The bending force is preferably simultaneously applied to parts (two locations) spaced apart from the center of the lightly-bent portion or the non-bent portion toward the width end of the plate material by an amount of W/4 at the time of pressing of the preformed body, such that an offset in which the end surfaces greatly differ in the gap portion is not formed.

The forming center of the press die used in the pressing of the preformed body preferably matches with the width center of the preformed body at the time of pressing of the preformed body, such that it is possible to evenly bend a portion corresponding to the width end of the plate material in the gap portion of the open pipe on the left and right sides, and a large offset is not formed in the gap portion.

The preformed body is preferably held in a U-shaped posture and is supported at its lowermost end (the center in the widthwise direction of the preformed body), such that it is possible to symmetrically deform the preformed body on the boundary of the center in the widthwise direction, and it is possible to obtain an open pipe with high roundness.

The press die is preferably constituted by a pair of bending members interposing the preformed body therebetween, and a forming surface having a cross-sectional shape which does not come into contact with the lightly-bent portion or the non-bent portion during pressing of the preformed body is formed in the bending member. Thus, the forming reaction force is decreased, and it is possible to efficiently produce the steel pipe.

At least one of the bending members preferably has a circular arc surface having a width center matching an axis of symmetry of the press die, and a forming surface having a slope leading to each of both ends of the circular arc surface and directed toward the axis of symmetry of the press die, such that it is possible to obtain a steel pipe with high roundness without forming a step in the gap portion.

When the central angle of the circular arc surface is set to not less than 28°, and the angle between the inclined surface and the straight line intersecting with a straight line passing through the widthwise center of the circular arc forming surface is set to not less than 14°, at the time of pressing of the preformed body, it is possible to reliably extend the lightly-bent portion or the non-bent portion toward the outside.

The lightly-bent portion or the non-bent portion is preferably not restricted by the forming surface of the press die by setting the circular arc surface to have the diameter of not more than 1.2 times the diameter of the steel pipe to be produced at the time of pressing of the preformed body, whereby the forming reaction force can be decreased.

### BRIEF DISCRIPTION OF THE DRAWINGS

FIG. 1 is a diagram schematically illustrating a preferred punch and die used to form a preformed body having a U-shaped cross-section.
FIG. 2 is a diagram schematically illustrating a preferred press die used to form an open pipe.
FIG. 3 is a diagram illustrating a specific forming condition when forming a plate material into a preformed body having a U-shaped cross-section.
FIG. 4 is an enlarged diagram illustrating a cross-section of the preformed body having the U-shaped cross-section.
FIG. 5 is a diagram illustrating a state in which the preformed body having the U-shaped cross-section is pressed into an open pipe.
FIG. 6 is a graph showing a relation between an amount of roundness variation/an outer diameter and (a length of lightly-bent portion or non-bent portion)/a plate width.
FIG. 7 is a graph showing a relation between an opening (mm) of a gap portion and (a length of lightly-bent portion or the non-bent portion)/a plate width.
FIG. 8 is a graph showing a relation between an opening (mm) of the U-shaped cross-section and (a length of lightly-bent portion or the non-bent portion)/a plate width.
FIG. 9 is an enlarged diagram illustrating essential portions of an upper die.
FIG. 10 is a graph showing a relation between an angle θd of a forming surface of the upper die and a direction θf of force.
FIG. 11 is a diagram illustrating a biting situation of the upper die.
FIG. 12 is a diagram illustrating a state in which a gap is formed between the upper die and the preformed body.
FIG. 13 is a graph showing a relation between (a radius of the circular arc surface of the upper die / a radius of the steel pipe) and the residual index.
FIG. 14 is a graph showing a relation between (a radius of the circular arc surface of the lower die / a radius of the steel pipe) and (forming load/load when the lightly-bent portion or the non-bent portion is freely bent).
FIG. 15 is a diagram illustrating the contact situation between the upper die and the lower die.

### EMBODIMENTS FOR CARRYING OUT THE INVENTION

Hereinafter, the present invention will be more specifically described with reference to the drawings.

FIGs. 1 and 2 are diagrams schematically illustrating a preferred punch and die and a preferred press die, respectively, that are used in the practice of the method of producing a steel pipe according to the present invention.

The punch and die shown in FIG. 1 is used when forming a plate material into a preformed body having a U-shaped cross-section by bending the plate material along its widthwise direction, and the press die shown in FIG. 2 is used when forming the preformed body into an open pipe having a gap in the longitudinal direction by applying a bending force to the preformed body having the U-shaped cross-section.

Reference number 1 in FIG. 1 denotes a die disposed in a conveying path of the plate material S. The die 1 is configured with a pair of left and right rod-like members la and lb that supports the plate material S at two locations along its feeding direction and enables a change in an interval e between the rod-like members la and lb depending on the size of the steel pipe to be produced.

Moreover, reference number 2 denotes a punch which is movable in a direction of moving close to or away from the die 1. The punch 2 includes a punch tip 2a having a downward convex forming surface that comes into direct contact with the plate material S to bend the plate material S into a concave shape, and a punch support 2b that is connected to the rear (upper end) of the punch tip 2a with the same width thereof to support the punch tip 2a.

Although a specific structure of the punch support 2b is not illustrated, its upper end portion is connected to a driving device such as hydraulic cylinder, and the punch support 2b can apply a bending force to the punch tip 2a by the driving device. Further, reference number 3 denotes a roller for forming the conveying path of the plate material S.

Further, reference number 4 in FIG. 2 denotes an upper die (bending tool), and reference number 5 denotes a lower die which mates with the upper die 4 (bending tool). The preformed body (which has a U-shaped cross-section) formed by the die 1 and the punch 2 is located between the upper die 4 and the lower die 5, and a bending force is applied to the preformed body to form an open pipe.

The upper die 4 may have a circular arc surface 4a having a width center that matches the forming center (an axis of symmetry) thereof, and a forming surface (inclined surface) 4b connected to each of both ends of the circular arc surface 4a and having a slope directed toward the forming center side of the press die. The lower die 5 may have a forming surface that does not come into contact with the lightly-bent portion or the non-bent portion during pressing of the preformed body. Further, the upper die 4 may have a press die having a forming surface that does not come into contact with the lightly-bent portion or the non-bent portion during pressing of the preformed body. As the lower die 5, it is possible to apply one that includes a circular arc surface having a width center matching the forming center (an axis of symmetry) thereof, and an inclined surface which is connected to each of both ends of the circular arc surface and is directed toward the forming center side of the press die.

In order to form the plate material S as a starting material into a tubular shape, first, end bending (also referred to as crimping) is performed on the width end portion of the plate material S.

The end bending is performed on a plate width end portion that is harder to bend as compared to the case of performing the bending using the die 1 and the punch 2, and it is possible to obtain a steel pipe in which high roundness is secured by providing an end bending portion by this forming.

Further, the roundness of the steel pipe is an indicator that indicates how much the cross-sectional shape of the steel pipe is close to a circle. Specifically, for example, when the produced steel pipe is equally divided into twelve sections or twenty-four sections in the circumferential direction at any pipe length position to measure the outer diameters at the opposite positions, and a maximum diameter and a minimum diameter thereof is defined by Dₘₐₓ and Dₘᵢₙ, respectively, the roundness = Dₘₐₓ - Dₘᵢₙ is defined. This indicates that as the roundness comes closer to 0, the cross-sectional shape of the steel pipe has a shape that is closer to a perfect circle.

The plate material S provided with the end bending portion is mounted on the die 1 as shown FIG. 1, and bending (3-point bending) is applied over the entire region as illustrated in FIG. 3, while intermittently feeding the plate material S by a predetermined feed amount, thereby forming the plate material into a preformed body which has a U-shaped cross-section as a whole.

Around a portion of the preformed body S₁ obtained by the bending, especially, a part each spaced apart from the width end portion by amount of W/4, a lightly-bent portion to which a slighter curvature is applied as compared to other regions or a non-bent portion P in which the bending is omitted is provided as shown in Fig. 4 by enlarging its cross-section.

The lightly-bent portion P can be provided by pressing while decreasing the bending amount applied by the punch 2, and the non-bent portion P can be provided by omitting the bending of the punch 2 while increasing the feeding of the plate material S.

Further, FIG. 3 specifically illustrates an example of a case of performing the bending and the feeding of the plate material S on the plate material S previously subjected to edge bending, sequentially from the top to the bottom of the left column, from the top to the bottom of the center column, and further from the top to the bottom of the right column, and the arrow assigned to each of the punch 2 and the plate material S in FIG. 3 illustrates the moving direction of the punch 2 and the plate material S at each stage.

As the punch 2 which performs bending on the plate material S, it is possible to use, for example, a punch having a substantially inverted T-shape in which the width of the punch tip 2a is larger than the width (thickness) of the punch support 2b. In this case, it is possible to bend a larger area with respect to the plate material by single step bending as compared to the configuration in which the width of the punch tip 2a is almost the same as the width (thickness) of the punch support 2b illustrated in FIG. 1, whereby the bending times can be decreased.

After a preformed body S₁ having a U-shaped cross-section is obtained, in order to form the preformed body S₁ into an open pipe, the preformed body S₁ is pressed using the upper die 4 and the lower die 5 illustrated in FIG. 2.

At the time of pressing of the preformed body S₁, the preformed body S₁ is held in a U-shaped posture so that an opening portion faces upward, and is located on the lower die 5 so that its lowest end, that is, the center in the widthwise direction becomes a support part. Thus, as illustrated in FIG. 5, the bending force is simultaneously applied to two locations of the width end portions of the plate material S which are parts spaced apart from the lightly-bent portion or the non-bent portion P toward the width end by amount of W/4 by the upper die 4.

In such pressing, since the preformed body S₁ is supported on the lower die 5 at a part at least away from the line of action of the bending force, and the lightly-bent portion or the non-bent portion P is not constrained by the press die, the preformed body S₁ is formed into a tubular shape without requiring excessive bending force.

As the lower die 5, in the present invention, although one having a forming surface that does not constrain the lightly-bent portion or the non-bent portion P is used, when the forming surface is a circular arc surface having a concave shape, it can be achieved by setting a larger diameter than the diameter of the steel pipe to be produced. Further, the forming surface may be a flat surface with which the preformed body S₁ linearly comes into contact.

In the stage of pressing the preformed body S₁ into an open pipe of the present invention, the bending force is applied at least to a part away from the center of the lightly-bent portion or the non-bent portion P by amount of W/4, the reason of which is as follows.

That is, the bending moment (M) when the whole preformed body S₁ has a circular shape is F·r ·cos *φ* (F: bending force, r: radius of circle) at a position of an angle *φ* from the position applied with the bending force, and becomes maximum at the position away from the position applied with the bending force by 90°, and the deformation also becomes maximum. Therefore, by applying the bending force to the position away from the center of the lightly-bent portion or the non-bent portion P by 90°, that is, 1/4 of the entire circumference, the lightly-bent portion or the non-bent portion P is effectively deformed. At this time, the bending moment is maximum at the position away from the applying position of the bending force by 90° and it becomes smaller as going away from this position. In order to allow the sufficient plastic deformation to occur in the lightly-bent portion or the non-bent portion P, the bending force is preferably applied by amount of W/4 ± 0.07 W.

Further, in the present invention, the center of the lightly-bent portion or the non-bent portion P is provided in a part including a part away from the width end portion of the plate material S by amount of W/4, the reason of which is as follows.

That is, as described above, although the bending force is preferably applied to a position apart from the center of the lightly-bent portion or the non-bent portion P in the width end direction of the plate material by amount of W/4, since its shape is changed at the step of forming the preformed body S₁ into an open pipe, a contact position with the upper die 4 is changed, and the position applied with the bending force is also changed. When the lightly-bent portion or the non-bent portion P is provided at a position spaced apart from the width end portion of the plate material S by amount of W/4, a position applied with the bending force is always a width end portion of the plate material S, and the lightly-bent portion or the non-bent portion P are most deformed. Thus, it is possible to give deformation to the lightly-bent portion or the non-bent portion P by single bending without changing the bending position. Further, in order to give a sufficient deformation to the lightly-bent portion or the non-bent portion P, the lightly-bent portion or the non-bent portion P is preferably provided in a range of W/4± 0.07W from the position applied with the bending force, that is, the width end portion of the plate material.

In the present invention, when the lightly-bent portion is provided in a part of the plate material S, particularly, in a part including the part away from the width end portion of the plate material S by amount of W/4, or when the non-bent portion P in which bending is omitted is provided in bending the plate material S , the length L (see FIG. 4) along the widthwise direction of the plate material S of the lightly-bent portion or the non-bent portion P is preferably set to not more than 10% of the plate width. The reason is as follows.

That is, when applying the bending force to the preformed body S₁ of a U-shaped cross-section having the lightly-bent portion or the non-bent portion P of the length L at the part spaced apart from the lightly-bent portion or the non-bent portion P by amount of W/4, bending moment acts on the lightly-bent portion or the non-bent portion P, and the portion is deformed.

The bending moment (M) when the whole preformed body S₁ becomes a circular shape is F ·r ·cos *φ* (F: bending force, r: radius of circle) at the position of the angle *φ* from the position applied with the bending force, and bending moment becomes maximum at the position spaced apart from the position applied with the bending force by 90°, and the amount of deformation is also the maximum. However, the amount of deformation is not uniform in the lightly-bent portion and the non-bent portion P. Therefore, the obtained open pipe has irregularities, rather than a uniform circular arc.

Here, as for a tubular material of an API standard Gr. X65 and a thickness of 38.1 mm, a relation between a value obtained by dividing the length L of the lightly-bent portion or the non-bent portion P of the shaped body S₁ having the U-shaped cross-section by the plate width and a value obtained by dividing an irregularity amount by the outer diameter of the tubular material is investigated. As illustrated in FIG. 6, as the length of the lightly-bent portion or the non-bent portion P is longer and the outer diameter is smaller, the irregularity amount is also larger. In the tubular material having the outer diameter of 559 mm, when the length of the lightly-bent portion or the non-bent portion P exceeds 10% of the plate width, the irregularity amount exceeds 1.5% of the outer diameter.

In the API standard which is a general standard of the line pipe, although the shape correction of a tube expansion ratio (rate for expanding the diameter) of about 1.5% is observed in the tube expanding process after joining (welding) the gap portion, when the irregularity amount exceeds 1.5% of the outer diameter, the dimensional accuracy of the finished product may be impaired. Therefore, in the present invention, the length L of the lightly-bent portion or the non-bent portion P along the widthwise direction of the plate material S is preferably set to not more than 10% of the plate width. Furthermore, in order to provide sufficient deformation to the lightly-bent portion or the non-bent portion P, the length L is preferably in the range of W/4± 0.07 W from the position applied with the bending force.

Further, when the length L of the lightly-bent portion or the non-bent portion P becomes longer, the difference in the gap portion of the open pipe increases by the spring back when releasing the bending force as illustrated in FIG. 7 and the butt-joining between the end surfaces may become difficult, which may cause restriction in some cases.

FIG. 8 is a graph showing a relation between the interval (opening of U-shaped cross-section) of the opening portion of the preformed body S₁ having a U-shaped cross-section and the length L of the lightly-bent portion or the non-bent portion P. Although the dimensional accuracy is better as the length L of the lightly-bent portion or the non-bent portion P becomes smaller, since the opening interval of the preformed body S₁ also becomes smaller, when the opening interval is smaller than the width of the punch 2, it is not possible to raise the punch 2 after the final bending (the last state of FIG. 3), and it is difficult to detach the preformed body S₁ from the press machine. Therefore, the lower limit of the length L is set depending on the size of the applied device or the steel pipe to be produced. For example, when a pipe having an outer diameter of 559 mm is produced by a press machine having the punch 2 having a width of 150 mm, L/W is required to be not less than 0.05.

In the present invention, when the opening angle defined based on the part on which the preformed body S₁ is supported is defined as θs, and the angle of the bending force applied to the preformed body S₁ is defined as θf, the pressing of the preformed body S₁ is started under a condition of θf > θs. However, the part in which the preformed body S₁ is supported by satisfying this condition is not existent on the line of action of the bending force, and the lightly-bent portion or the non-bent portion P can reliably extend toward the outside with relatively small bending force.

Further, when the widthwise center of the preformed body is located at the lowermost end (part on which the preformed body is supported) in the U-shaped posture in which the opening portion of the preformed body is located upward, and the straight line q which symmetrically bisects the preformed body through the widthwise center is defined as a reference line, the opening angle θs of the preformed body S₁ is defined as an angle formed between the reference line and the straight line r connecting the widthwise center (W/2) of the preformed body and the widthwise end portion of the preformed body S₁ (see FIG. 5). Further, the angle (direction of the bending force) θf of the bending force is determined by the press die shape and the friction coefficient, when the angle (angle to the horizontal plane) of the forming surface of the press die is defined as θd, and the friction coefficient of the press die surface is defined as µ, the angle θf is determined as θf = θd - tan⁻¹ (µ) (see FIG. 9).

When the forming surface of the upper die 4 is configured to include a circular arc surface 4a having a width center that matches the forming center O of the press die, and a pair of forming surfaces 4b which is connected to each of both ends of the circular arc surface 4a and is directed toward the forming center O side of the press die, the forming surfaces 4b may be a straight inclined surface or a curved inclined surface.

The central angle θc of the circular arc surface 4a is set in the range of not less than 28°, and the forming surface 4b is deformed so as to reliably extend the lightly-bent portion or the non-bent portion P to the outside at the time of pressing of the preformed body S₁. Therefore, it is possible to set the angle θd formed with the straight line intersecting with the straight line passing through the widthwise center of the circular arc surface 4a in the range of not less than 14° (see FIG. 2).

The reason of desirably setting the central angle 0c of the circular arc surface 4a of the upper die 4 to not less than 28° is as follows. FIG. 10 illustrates the result of a relation between the angle 0d of the forming surface 4b of the upper die 4 and the direction θf (angle of the bending force) of force obtained for a general lubrication state (the case of the friction coefficient of 0.1).

As seen from FIG. 10, the larger the angle θd of the forming surface of the upper die 4 is, the larger the direction θF of force is, and lightly-bent portion or the non-bent portion P easily extends outward. For example, when a pipe having an outer diameter of 559 mm is produced by a press machine having the width of the punch 2 of 150 mm (an example of a minimum dimension of paragraph (0055)), the minimum value of L/W is 0.05, and the opening angle θs of the preformed body S₁ is 9°. At this time, if the press die angle θd is not less than 14°, the direction θf of power is larger than the opening angle θs of the preformed body S₁. In addition, the opening angle θs of the preformed body S₁ is geometrically determined by the ratio of the length L and the plate width W of the lightly-bent portion or the non-bent portion P, and when the L/W increases, the opening angle θs of the preformed body S₁ also increases. Thus, in some cases, it may be necessary to further increase the central angle 0c of the circular arc surface 4a of the upper die 4.

Meanwhile, when the angle θd of the forming surface 4b of the upper die 4 is large, the opening portion of the press die becomes smaller than the maximum width of the preformed body S₁ having a U-shaped cross-section, and as illustrated in FIG. 11, since the upper die 4 may bite into the preformed body S₁ and scratch it, its upper limit is determined depending on a maximum width of the preformed body S₁.

At the time of pressing of the preformed body S₁, when the bending force is simultaneously applied to each of the parts (two locations) spaced apart from the lightly-bent portion or the non-bent portion P toward the width end (width end of the preformed body S₁) of the plate material S by amount of W/4, it is effective to mate the forming center O of the press die used for the pressing of the preformed body S₁ with the widthwise center W/2 of the preformed body S₁, whereby an occurrence of a step difference (offset) in the gap portion of the open pipe S₂ can be avoided.

The circular arc surface 4a of the upper die 4 may be set to the radius of not more than 1.2 times the diameter of the steel pipe to be produced. The reason is as follows.

When the radius of the circular arc surface 4a of the upper die 4 is small, as illustrated in FIG. 12, a space is formed between the upper die 4 and the preformed body S₁ during forming, there is a risk of mis-alignment of the end surface in the gap portion, and its lower limit is defined depending on the shape near the plate end defined by the end bending so that the contact is possible in the range of about the plate thickness from the plate end.

FIG. 13 shows a relation between (the radius of circular arc surface 4a of the upper die 4/ the radius of the steel pipe) and the index (residual index) in which the lightly-bent portion or the non-bent portion P is left (not bent to circular) as it is. When the radius of the circular arc surface 4a of the upper die 4 increases, the restriction is insufficient, and thus, the lightly-bent portion or the non-bent portion P remains as it is. When the residual index 1.0 is defined as a reference value, in order not to exceed the reference value, the radius of the circular arc surface 4a of the upper die 4 is desirably suppressed to not more than 1.2 times the radius of the steel pipe to be produced.

Next, when the lower die 5a has a circular arc surface 5a in which a forming surface has a concave shape, as illustrated in Fig. 5, there is a need to use one larger than the external diameter of the steel pipe to be produced so that the preformed body S₁ having a U-shaped cross-section fits into the press die.

FIG. 14 is a graph showing a relation between (the radius of the circular arc surface 5a of the lower die 5/the radius of the steel pipe) and (the forming load/the load when the lightly-bent portion or the non-bent portion P is freely bent). When the radius of the circular arc surface 5a of the lower die 5 is small, since the lightly-bent portion or the non-bent portion P is restricted by the press die during forming of the preformed body S₁, the forming load increases. In particular, when the radius of the circular arc surface 5a of the lower die 5 is less than 1.05 times the diameter of the steel pipe to be produced, the forming load rapidly increases. Therefore, the radius of the circular arc surface 5a of the lower die 5 is desirably not less than 1.05 times the diameter of the steel pipe to be produced. When the radius of the circular arc surface 5a of the lower die 5 is set to not less than 1.07 times the diameter of the steel pipe to be produced, it can be suppressed to not more than twice of the load applied when forming the preformed body S₁ in a non-restriction state.

When the radius of the circular arc surface 5a of the lower die 5 is large, as illustrated in FIG. 15, since the contact with the upper die 4 is unavoidable, a desired pressing rate is not attained, the deformation of the lightly-bent portion or the non-bent portion P may be insufficient or the opening amount of the gap portion may increase, so that it is necessary to select the lower die 5 depending on the shape of the upper die 4. When using the lower die 5 having the circular arc surface 5a having the concave shape, it is possible to directly use the die used when producing the steel pipe by the UO method without any change, and there is no need for producing the die. However, as long as it is possible to avoid the restrictions of the lightly-bent portion or the non-bent portion P, those having the same configuration as the upper die 4 may be applied.

Further, although an example in which the forming surface (inclined surface) 4b is made up of a circular arc surface 4a and the forming surface (inclined surface) 4b is adopted as the upper die 4, as long as it is possible to satisfy the condition θs > θf at the time of starting of pressing, a press die equipped with a forming surface formed with the circular arc surface 5a such as the lower die 5 may be used, and is not limited to the illustrated configuration.

As the lower die 5, it is possible to use one such as die 1 illustrated in FIG. 1 which supports the preformed body S₁ at two points or a roller-type die. Even when using the die, since the lightly-bent portion or the non-bent portion P is not restricted by the forming surface of the press die during pressing, the preformed body S₁ can be formed into a tubular shape with a relatively small bending force.

Thereafter, the open pipe S₂ obtained by pressing using the upper die 4 and the lower die 5 mutually abuts the end surfaces of the gap portion, is welded by a welding machine (a joining means) and is further formed into a steel pipe by being expanded as required.

As the welding machine (a joining means), for example, a welding machine made up of three kinds of welding machines, such as a tack welding machine, an inner surface welding machine and an outer surface welding machine, is applied. In the welding machine, the tack welding machine continuously brings the butted surfaces into close contact with each other at the appropriate positional relation by cage rolls, and welds the close-contact portions over its entire length.

Next, the tack pipe is welded (submerged arc welding) from the inner surface of the butted portion by the inner surface welding machine, and is further welded (submerged arc welding) from the outer surface of the butted portion by the outer surface welding machine.

The positional relation between the welding machine (the joining means) and the press die (the upper die 4 and the lower die 5) for pressing the preformed body S₁ is not particularly limited, and can be arbitrarily changed.

### EXAMPLE 1

In order to form the steel pipe with a diameter of 91.44 cm (36 inches) using a line pipe steel plate(API grade X60) having a thickness of 38.1 mm and a width of 2711 mm, the material is placed on a die in which an interval of a rod-like member is set to 450 mm, and bending of the three-point bending is performed from the position of 1120 mm from the width center of the plate material, with a plate material feeding pitch of 224 mm and 11 bending times (five times from the paper right end, and five times from the left end) by a punch having a forming surface of a radius of 308 mm. At that time, the bending amount is set to an amount in which the punch tip reaches a position of 15.8 mm from the line connecting the uppermost part of the rod-like member, and bending is performed by 30° for a time. However, at the position of 672 mm from the width center of the plate material (at the time of third feeding from the right end, and third feeding from the left end), the bending is not performed, and the non-bent portion is formed at the position of 571 to 795 mm. Next, while holding the preformed body having the U-shaped cross-section obtained by bending in a U-shaped posture so that the opening portion faces upward, when pressing the preformed body into an open pipe until an inter-apex distance (the apex of the R part is an uppermost part of the circular arc surface in the upper die, and a lowermost part of the circular arc surface in the lower die) of a R part of the press die reaches 880 mm, using an upper die having a circular arc surface of a radius R: 457.2 mm and a central angle θc: 60° and a flat surface leading to the circular arc surface at the angle θd: 30° and a lower die having a concave circular arc surface of a radius R: 502.9 mm, the degree of the decrease of the bending force of the press die, the opening amount in the gap portion of the open pipe, the amount of offset, and the roundness of the steel pipe after welding are investigated.

As a result, after performing the U-shape press at a standard condition, by performing the O-shape press at the compression ratio of 0.2% using a press die of the radius R: 452.6 mm, as a result of being compared to the case (conventional method) of producing the steel pipe of an outer diameter of 36 inches and a thickness (wall thickness) of 38.1 mm, when producing the steel pipe according to the present invention, it is confirmed that the bending force of the O-shape press is decreased to about 15% as compared to the conventional method.

In addition, it becomes clear that the steel pipe can be obtained in which the opening amount in the gap portion of the open pipe is 21 mm, the amount of offset after welding (steel pipe) is 0.1 mm, the roundness is 5.2 mm and a difference to an outer diameter of 91.44 cm (36 inches) is only 0.6%.

### EXAMPLE 2

As in Example 1, in order to form a steel pipe with a diameter of 91.44 cm (36 inches) using a line pipe steel plate(API grade X60) having a thickness of 38.1 mm and a width of 2711 mm, the material is placed on a die in which an interval of a rod-like member is set to 450 mm, and bending of the three-point bending is performed by 30° for a time, from the position of 1120 mm from the width center of the plate material, with a plate material feeding pitch of 224 mm and 11 bending times (five times from the paper right end, and five times from the left end) by a punch having a forming surface of a radius of 308 mm. At that time, the bending amount is set to an amount in which the punch tip reaches a position of 15.8 mm from the line connecting the uppermost part of the rod-like member, and bending is performed by 30° for a time. However, at the position of 672 mm from the width center of the plate material (at the time of third feeding from the right end, and third feeding from the left end), the lightly-bent portion is formed at the position of 571 to 795 mm, while decreasing the bending amount to 8.8 mm and performing the bending of 10°.

Next, while holding the preformed body having the U-shaped cross-section obtained by bending in a U-shaped posture so that the opening portion faces upward, when pressing the preformed body into an open pipe until an inter-apex distance (the apex of the R part is the uppermost part of the circular arc surface in the upper die, and the lowermost part of the circular arc surface in the lower die) of the R part of the press die reaches 880 mm, using the upper die having a circular arc surface of a radius R: 457.2 mm and a central angle θc: 60° and a flat surface leading to the circular arc surface at the angle θd: 30°, and the lower die having a concave circular arc surface of a radius R: 502.9 mm, the degree of pressing of the bending force of the press die, the opening amount in the gap portion of the open pipe, the amount of offset, and the roundness of the steel pipe after welding are investigated.

As a result, after performing the U-shape press at a standard condition, by performing the O-shape press at the compression ratio of 0.2% using a press die of the radius R: 452.6 mm, as a result of being compared to the case (conventional method) of producing the steel pipe of an outer diameter of 91.44 cm (36 inches) and a thickness (wall thickness) of 38.1 mm, when producing the steel pipe according to the present invention, it is confirmed that the bending force of the O-shape press is decreased to about 15% as compared to the conventional method.

Further, it becomes clear that the steel pipe can be obtained in which the opening amount in the gap portion of the open pipe is 16 mm, the amount of offset after welding (in steel pipe) is 0.1 mm, the roundness is 8.2 mm, and a difference to an outer diameter of 91.44 cm (36 inches) is only about 0.9%.

### EXAMPLE 3

In order to form a steel pipe with a diameter of 106.68 cm (42 inches) using a line pipe steel plate(API grade X80) having a thickness of 44.5 mm, a width of 3180 mm and a length of 12.2 mm, the material is placed on the die in which the interval of the rod-like members is set to 500 mm, and bending of the three-point bending is performed by a punch having a forming surface with a radius of 360 mm, and a preformed body having a U-shaped cross-section with different position and length of the non-bent portion from the width end portion is prepared.

Next, the lower die having a concave circular arc surface having a radius R: 609.6 mm is installed on the rod-like member, and the preformed body having the U-shaped cross-section obtained by bending is pressed from the outside into an open pipe until an inter-apex distance (the apex of the R part is the uppermost part of the circular arc surface in the upper die, and the lowermost part of the circular arc surface in the lower die) of the R part of the press die reaches 1027 mm.

In the case of pressing the preformed body into the open pipe, the bending force of the press die, the opening amount and the amount of offset in the gap portion of the open pipe, and the roundness of the steel pipe after welding are investigated. The results are shown in Table 1 together with the bent position and the shape of the preformed body.

**Table 1**

| No | Press condition | Shape of preformed body | | Index of press condition (ratio to plate width) | | | Result | | | |
|---|---|---|---|---|---|---|---|---|---|---|
| | Bending force addition position [mm] | Center position of non-bent portion [mm] | Length of non-bent portion [mm] | Distance between bending force addition position and center of non-bent portion | Center position of non-bent portion | Length of non-bent portion | Load [MN] | Roundness [mm] | Amount of offset [mm] | Opening [mm] |
| 1 | 477 | 986 | 318 | 0.16 | 0.31 | 0.10 | 27 | 18.1 | 1.5 | 60 |
| 2 | 382 | 986 | 318 | 0.19 | 0.31 | 0.10 | 23 | 13.9 | 0.8 | 50 |
| 3 | 286 | 986 | 318 | 0.22 | 0.31 | 0.10 | 20 | 8.5 | 0.9 | 80 |
| 4 | 191 | 986 | 318 | 0.25 | 0.31 | 0.10 | 18 | 7.5 | 0.6 | 100 |
| 5 | 95 | 986 | 318 | 0.28 | 0.31 | 0.10 | 16 | 10.7 | 0.8 | 120 |
| 6 | 0 | 986 | 318 | 0.31 | 0.31 | 0.10 | 15 | 13.9 | 1.0 | 150 |
| 7 | 95 | 890 | 318 | 0.25 | 0.28 | 0.10 | 16 | 10.7 | 0.6 | 90 |
| 8 | 0 | 795 | 318 | 0.25 | 0.25 | 0.10 | 17 | 5.3 | 0.7 | 80 |
| 9 | 0 | 700 | 318 | 0.22 | 0.22 | 0.10 | 20 | 9.6 | 0.5 | 120 |
| 10 | 0 | 604 | 318 | 0.19 | 0.19 | 0.10 | 23 | 14.9 | 0.7 | 100 |
| 11 | 0 | 509 | 318 | 0.16 | 0.16 | 0.10 | 28 | 17.1 | 1.0 | 110 |
| 12 | 0 | 795 | 127 | 0.25 | 0.25 | 0.04 | 17 | 7.5 | 0.2 | 60 |
| 13 | 0 | 795 | 191 | 0.25 | 0.25 | 0.06 | 18 | 9.1 | 0.5 | 70 |
| 14 | 0 | 795 | 254 | 0.25 | 0.25 | 0.08 | 18 | 11.2 | 0.7 | 80 |
| 15 | 0 | 795 | 382 | 0.25 | 0.25 | 0.12 | 18 | 10.1 | 1.0 | 120 |
| 16 | 0 | 795 | 445 | 0.25 | 0.25 | 0.14 | 19 | 19.2 | 0.9 | 140 |

As in Nos. 2 to 6, when adding the bending force to a position spaced apart from the center of the non-bent portion by 0.19 to 0.31 of the plate width, the roundness and the amount of offset are good. However, in No. 1 of 0.16 which is close to the non-bent portion, the roundness is 18.1 mm which exceeds 1.5 % of the product diameter, and the amount of offset is also 1.5 mm which is larger than the other cases.

In addition, as the addition position of the bending force is away from the non-bent portion, the bending force becomes smaller.

In addition, as in Nos. 7 to 10, when setting the non-bent portion from the plate width end portion in the range of 0.28 to 0.19, the satisfactory roundness is obtained, but in No. 11 in which the non-bent portion is close to the plate width end portion, the roundness is 17.1 mm which exceeds 1.5% of the product diameter.

In addition, as in Nos. 12 to 15, when the length of the non-bent portion is not more than 0.12 of the plate width, the satisfactory roundness is obtained, but in No. 16 in which the length of the non-bent portion is large, the roundness is 19.2 mm which exceeds 1.5% of the product diameter.

### EXAMPLE 4

In order to form a steel pipe with a diameter of 106.68 cm (42 inches) using a line pipe steel plate(API grade X80) having a thickness of 44.5 mm, a width of 3180 mm and a length of 12.2 mm, the material is placed on the die in which the interval of the rod-like members is set to 500 mm, and bending of the three-point bending is performed by a punch having a forming surface with a radius of 360 mm, and a preformed body having a U-shaped cross-section with different position and length of the non-bent portion from the width end portion is prepared.

Next, while holding the preformed body having the U-shaped cross-section obtained by bending in a U-shaped posture so that the opening portion faces upward, when pressing the preformed body into an open pipe, until an inter-apex distance (the apex of the R part is the uppermost part of the circular arc surface in the upper die, and the lowermost part of the circular arc surface in the lower die) of the R part of the press die reaches 1027 mm, using the upper die having a circular arc surface of a radius R: 533.4 mm and a central angle θc: 60° and a flat surface leading to the circular arc surface at the angle ed: 30°, and the lower die having a concave circular arc surface of a radius R: 609.6 mm, in the state that the upper die is in contact with both plate width end portions, the degree of pressing of the bending force of the press die, the opening amount in the gap portion of the open pipe, the amount of offset, and the roundness of the steel pipe after welding are investigated. The results are shown in Table 2 together with the bent position and the shape of the preformed body. The same shapes as in Example 3 are denoted by the same No.

**Table 2**

| No | Press condition | Shape of preformed body | | Index of press condition (ratio to plate width) | | | Result | | | |
|---|---|---|---|---|---|---|---|---|---|---|
| | Bending force addition position [mm] | Center position of non-bent portion [mm] | Length of non-bent portion [mm] | Distance between bending force addition position and center of non-bent portion | Center position of non-bent portion | Length of bent portion | Load [MN] | 1 Roundness [mm] | Amount of offset [mm] | Opening [mm] |
| 7 | 0 | 890 | 318 | 0.28 | 0.28 | 0.10 | 32 | 8.0 | 0.2 | 110 |
| 8 | 0 | 795 | 318 | 0.25 | 0.25 | 0.10 | 36 | 4.3 | 0.1 | 100 |
| 9 | 0 | 700 | 318 | 0.22 | 0.22 | 0.10 | 40 | 8.5 | 0.1 | 90 |
| 10 | 0 | 604 | 318 | 0.19 | 0.19 | 0.10 | 47 | 11.2 | 0.2 | 100 |
| 11 | 0 | 509 | 318 | 0.16 | 0.16 | 0.10 | 56 | 16.5 | 0.1 | 80 |
| 12 | 0 | 795 | 127 | 0.25 | 0.25 | 0.04 | 35 | 6.4 | 0.1 | 70 |
| 13 | 0 | 795 | 191 | 0.25 | 0.25 | 0.06 | 35 | 5.9 | 0.0 | 70 |
| 14 | 0 | 795 | 254 | 0.25 | 0.25 | 0.08 | 36 | 5.3 | 0.1 | 90 |
| 15 | 0 | 795 | 382 | 0.25 | 0.25 | 0.12 | 37 | 6.4 | 0.2 | 130 |
| 16 | 0 | 795 | 445 | 0.25 | 0.25 | 0.14 | 37 | 17.1 | 0.1 | 140 |

As in Nos. 7 to 10, when setting the non-bent portion from the plate width end portion within the range of 0.28 to 0.19, the satisfactory roundness is obtained. However, in No. 11 in which the non-bent portion is close to the plate width end portion, the roundness is 16.5 mm which exceeds 1.5% of the product diameter.

In addition, as in No. 12 to 15, when the length of the non-bent portion is not more than 0.12 of the plate width, the satisfactory roundness is obtained. However, in No. 16 in which the length of the non-bent portion is large, the roundness is 17.1 mm which exceeds 1.5% of the product diameter. Furthermore, all the amount of offset is not more than 0.2 mm which is smaller than in Example 3 performing the bending one side by one side.

### EXAMPLE 5

In order to form a steel pipe with a diameter of 55.88 cm (22 inches) using a line pipe steel plate(API grade X80) having a thickness of 31.8 mm, a width of 1640 mm and a length of 12.2 mm, the material is placed on the die in which the interval of the rod-like members is set to 400 mm, and bending of the three-point bending is performed by a punch having a forming surface with a radius of 188 mm, and a preformed body having a U-shaped cross-section with different position and length of the non-bent portion from the width end portion is prepared.

Next, a lower die having a concave circular arc surface having a radius R: 330.2 mm is installed on the rod-like member, and the preformed body having the U-shaped cross-section obtained by bending is pressed from the outside into an open pipe, until an inter-apex distance (the apex of the R part is the uppermost part of the circular arc surface in the upper die, and the lowermost part of the circular arc surface in the lower die) of the R part of the press die reaches 538 mm,

In the case of pressing the preformed body into the open pipe, the bending force of the press die, the opening amount and the amount of offset in the gap portion of the open pipe, and the roundness of the steel pipe after welding are investigated. The results are described in Table 3 together with the bent position and the shape of the preformed body.

**Table 3**

| No | Press condition | Shape of preformed body | | Index of press condition (ratio to plate width) | | | Result | | | |
|---|---|---|---|---|---|---|---|---|---|---|
| | Bending force addition position [mm] | Center position of non-bent portion [mm] | Length of non-bent portion [mm] | Distance between bending force addition position and center of non-bent portion | Center position of non-bent portion | Length of non-bent portion | Load [MN] | Roundness [mm] | Amount of offset [mm] | Opening [mm] |
| 1 | 246 | 508 | 164 | 0.16 | 0.31 | 0.10 | 37 | 10.1 | 1.4 | 60 |
| 2 | 197 | 508 | 164 | 0.19 | 0.31 | 0.10 | 32 | 7.8 | 0.7 | 50 |
| 3 | 148 | 508 | 164 | 0.22 | 0.31 | 0.10 | 28 | 5.0 | 0.9 | 80 |
| 4 | 98 | 508 | 164 | 0.25 | 0.31 | 0.10 | 25 | 4.6 | 0.7 | 100 |
| 5 | 49 | 508 | 164 | 0.28 | 0.31 | 0.10 | 22 | 6.7 | 0.6 | 120 |
| 6 | 0 | 508 | 164 | 0.31 | 0.31 | 0.10 | 21 | 7.8 | 0.9 | 150 |
| 7 | 49 | 459 | 164 | 0.25 | 0.28 | 0.10 | 23 | 5.6 | 0.5 | 90 |
| 8 | 0 | 410 | 164 | 0.25 | 0.25 | 0.10 | 24 | 39 | 0.4 | 80 |
| 9 | 0 | 361 | 164 | 0.22 | 0.22 | 010 | 28 | 5.0 | 0.6 | 120 |
| 10 | 0 | 311 | 164 | 0.19 | 0.19 | 0.10 | 32 | 7.8 | 0.6 | 100 |
| 11 | 0 | 262 | 164 | 0.16 | 0.16 | 0.10 | 40 | 10.6 | 1.0 | 110 |
| 12 | 0 | 410 | 98 | 0.25 | 0.25 | 0.06 | 25 | 5.0 | 0.5 | 70 |
| 13 | 0 | 410 | 131 | 0.25 | 0.25 | 0.08 | 26 | 56 | 0.9 | 80 |
| 14 | 0 | 410 | 197 | 0.25 | 0.25 | 0.12 | 26 | 53 | 0.9 | 120 |
| 15 | 0 | 410 | 229 | 0.25 | 0.25 | 0 14 | 26 | 11.2 | 1.1 | 140 |

As in Nos. 2 to 6, when adding the bending force to a position spaced apart from the center of the non-bent portion by 0.19 to 0.31 of the plate width, both the roundness and the amount of offset are good. However, in No. 1 of 0.16 which is close to the non-bent portion, the roundness is 10.1 mm which exceeds 1.5 % of the product diameter, and the amount of offset is 1.4 mm which is larger than the other cases.

Further, as the addition position of the bending force is away from the non-bent portion, the bending force becomes smaller. Further, as in Nos. 7 to 10, when providing the non-bent portion in the range of 0.28 to 0.19 from the plate width end portion, the satisfactory roundness is obtained, but in No. 11 in which the non-bent portion is close to the plate width end portion, the roundness is 10.6 mm which exceeds 1.5% of the product diameter. Furthermore, as in Nos. 12 to 14, when the length of the non-bent portion is not more than 0.12 of the plate width, the satisfactory roundness is obtained, but in No. 15 in which the length of the non-bent portion is large, the roundness is 11.2 mm which exceeds 1.5% of the product diameter.

### EXAMPLE 6

In order to form a steel pipe with a diameter of 55.88 cm (22 inches) using a line pipe steel plate(API grade X80) having a thickness of 31.8 mm, a width of 1640 mm and a length of 12.2 mm, the material is placed on the die in which the interval of the rod-like members is set to 400 mm, and bending of the three-point bending is performed by a punch having a forming surface with a radius of 188 mm, and a preformed body having a U-shaped cross-section with different position and length of the non-bent portion from the width end portion is prepared.

Next, while holding the preformed body having the U-shaped cross-section obtained by bending in a U-shaped posture so that the opening portion faces upward, when pressing the preformed body into an open pipe, until an inter-apex distance (the apex of the R part is the uppermost part of the circular arc surface in the upper die, and the lowermost part of the circular arc surface in the lower die) of the R part of the press die reaches 538 mm, using the upper die having a circular arc surface of a radius R: 279.4 mm and a central angle θc: 60° and a flat surface leading to the circular arc surface at the angle θd: 30°, and the lower die having a concave circular arc surface of a radius R: 330.2 mm, in the state that the upper die is in contact with both plate width end portions, the degree of pressing of the bending force of the press die, the opening amount in the gap portion of the open pipe, the amount of offset, and the roundness of the steel pipe after welding are investigated. The results are described in Table 4 together with the bent position and the shape of the preformed body. The same shapes as in Example 5 are denoted by the same No.

**Table 4**

| No | Press condition | Shape of preformed body | | Index of press condition (ratio to plate width) | | | Result | | | |
|---|---|---|---|---|---|---|---|---|---|---|
| | Bending force addition position [mm] | Center position of non-bent portion [mm] | Length of non-bent portion [mm] | Distance between bending force addition position .. and center of non-bent portion. | Center position of non-bent portion | Length of non-bent portion. | Load [MN] | Roundness [mm] | Amount of offset [mm] | Opening [mm] |
| 7 | 0 | 459 | 164 | 0.28 | 0.28 | 0.10 | 46 | 4.7 | 0.0 | 110 |
| 8 | 0 | 410 | 164 | 0.25 | 0.25 | 0.10 | 50 | 3.1 | 0.2 | 100 |
| 9 | 0 | 361 | 164 | 0.22 | 0.22 | 0.10 | 55 | 4.5 | 0.1 | 90 |
| 10 | 0 | 311 | 164 | 0.19 | 0.19 | 0.10 | 65 | 7.3 | 0.2 | 100 |
| 11 | 0 | 262 | 164 | 0.16 | 0.16 | 0.10 | 78 | 9.8 | 0.3 | 80 |
| 12 | 0 | 410 | 98 | 0.25 | 0.25 | 0.06 | 50 | 3.6 | 0.0 | 70 |
| 13 | 0 | 410 | 131 | 0.25 | 0.25 | 0.08 | 51 | 3.9 | 0.1 | 90 |
| 14 | 0 | 410 | 197 | 0.25 | 0.25 | 0.12 | 51 | 3.4 | 0.3 | 130 |
| 15 | 0 | 410 | 229 | 0.25 | 0.25 | 0.14 | 52 | 10.1 | 0.2 | 140 |

As in Nos. 7 to 10, when providing the non-bent portion within the range of 0.28 to 0.19 from the plate width end portion, the satisfactory roundness is obtained. However, in No. 11 in which the non-bent portion is close to the plate width end portion, the roundness is 9.8 mm which exceeds 1 .5% of the product diameter.

In addition, as in Nos. 12 to 14, when the length of the non-bent portion is not more than 0.12 of the plate width, the satisfactory roundness is obtained. However, in No. 15 in which the length of the non-bent portion is large, the roundness is 10.1 mm which exceeds 1.5% of the product diameter. Furthermore, all the amount of offset is not more than 0.3 mm which is smaller than in Example 3 performing bending one side by one side.

### EXAMPLE 7

In order to form a steel pipe with a diameter of 91.44 cm (36 inches) using a line pipe steel plate(API grade X60) having a thickness of 38.1 mm, a width of 2711 mm and a length of 12.2 mm, the material is placed on the die in which the interval of the rod-like members is set to 450 mm, and bending of the three-point bending is performed by a punch having a forming surface with a radius of 308 mm, and a preformed body having a U-shaped cross section provided with non-bent portions of the length of 109 mm and 224 mm around the position of 683 mm from the plate width end portion is prepared.

Next, while holding the preformed body having the U-shaped cross-section obtained by bending in a U-shaped posture so that the opening portion faces upward, when pressing the preformed body into an open pipe, until an inter-apex distance (the apex of the R part is the uppermost part of the circular arc surface in the upper die, and the lowermost part of the circular arc surface in the lower die) of the R part of the press die reaches 880 mm, using the upper die having a circular arc surface of a radius R: 457.2 mm and various central angles and a flat surface leading to the circular arc surface, and the lower die having a concave circular arc surface of a radius R: 502.9 mm, in the state that the upper die is in contact with both plate width end portions, the degree of pressing of the bending force of the press die, the opening amount in the gap portion of the open pipe, and the roundness of the steel pipe after welding are investigated. Table 5 describes the results together with the length of the non-bent portion, the opening angle θs of the preformed body having the U-shaped cross-section, the central angle of the upper die and the angle θf of the bending force.

As in Nos. 3, 5 and 6, under the condition of θf > θs, the opening amount is also small and the roundness is also good. Meanwhile, in Nos. 1, 2 and 4 of θf < θs, the opening amount is large, and in Nos. 1 and 4, the opening amount is too large to perform the welding. In addition, although the welding can be performed in No. 2, the roundness is 15.7 mm which exceeds 1.5% of the product diameter.

### EXAMPLE 8

In order to form a steel pipe with various diameters of 28 to 96.52 cm (38 inches) using a line pipe steel plate (API grade X60) having a thickness of 38.1 mm and a length of 12.2 mm, bending of the three-point bending is performed, and a preformed body having a U-shaped cross section provided with a non-bent portion of 0.08 times the plate width around the position of W/4 from the plate width end portion is prepared.

Next, while holding the preformed body having the U-shaped cross-section obtained by bending in a U-shaped posture so that the opening portion faces upward, when pressing the preformed body into an open pipe, until an inter-apex distance (the apex of the R part is the uppermost part of the circular arc surface in the upper die, and the lowermost part of the circular arc surface in the lower die) of the R part of the press die reaches 0.96 times the outer diameter, using the upper die having a circular arc surface of a radius R: 457.2 mm and a central angle θc: 60° and various radiuses leading to the circular arc surface at the angle θd: 30°, and the lower die having a concave circular arc surface of a radius larger than the outer diameter by 50.8 mm, in the state that the upper die is in contact with both plate width end portions, the degree of pressing of the bending force of the press die, the amount of offset in the gap portion of the open pipe, and the roundness of the steel pipe after welding are investigated. Table 6 describes the results together with the outer diameter of the steel pipe, and the ratio of the radius of the upper die to the outer radius of the steel pipe.

**Table 6**

| No | Outer diameter of steel pipe [mm] | Radius of upper die/ outer radius of steel pipe | Roundness [mm] | Amount of offset [mm] |
|---|---|---|---|---|
| 1 | 965.2 | 0.95 | 5.7 | 1.0 |
| 2 | 914.4 | 1.00 | 5.2 | 0.2 |
| 3 | 863.6 | 1.06 | 6.2 | 0.1 |
| 4 | 812.8 | 1.13 | 8.3 | 0.2 |
| 5 | 762.0 | 1.20 | 10.2 | 0.3 |
| 6 | 711.2 | 1.29 | 17.2 | 0.2 |

In Nos. 1 to 5 in which the ratio of the radius of the upper die to the outer radius of the steel pipe is not more than 1.2, the roundness is good, and smaller the ratio is, the better the roundness is. In addition, in No. 1 in which the radius of the upper die is smaller than the outer radius of the steel pipe, the amount of offset is larger than Nos. 2 to 5 in which the ratio is not less than 1.0. Meanwhile, in No. 6 in which ratio of the radius of the upper die to the outer radius of the steel pipe is large, the roundness is 17.2 mm which exceeds 1.5% of the product diameter.

### EXAMPLE 9

In order to form a steel pipe with a diameter of 91.44 cm (36 inches)using a line pipe steel plate (API grade X60) having a thickness of 38.1 mm, a width of 2711 mm and a length of 12.2 mm, the material is placed on the die in which the interval of the rod-like members is set to 450 mm, and bending of the three-point 25 bending is performed by a punch having a forming surface with a radius of 308 mm, and a preformed body having a U-shaped cross section provided with a non-bent portion of the length of 224 mm around the position of 683 mm from the plate width end portion is prepared.

Next, while holding the preformed body having the U-shaped cross-section obtained by bending in a U-shaped posture so that the opening portion faces upward, when pressing the preformed body into an open pipe, until an inter-apex distance (the apex of the R part is the uppermost part of the circular arc surface in the upper die, and the lowermost part of the circular arc surface in the lower die) of the R part of the press die reaches 880 mm, using the upper die having a circular arc surface of a radius R: 457.2 mm and a central angle 6c: 60° and various radiuses R leading to the circular arc surface at the angle θd: 30°, and the lower die having a concave circular arc surface of various radiuses, in the state that the upper die is in contact with both plate width end portions, the bending force (load) of the press die is investigated. Table 7 describes a relation among deformation of the lower die, a ratio to the outer radius of the steel pipe, and the bending force.

**Table 7**

| No | Radius of lower die [mm] | Radius of lower die / outer radius of steel pipe | Load [MN] |
|---|---|---|---|
| 1 | 482.6 | 1.06 | 75 |
| 2 | 508.0 | 1.11 | 50 |
| 3 | 533.4 | 1.17 | 35 |
| 4 | 558.8 | 1.22 | 35 |

As the radius of the lower die is increased, its load is decreased. In Nos. 3 and 4 in which the ratio is in excess of 1.15, there is no contact with the press die, and the load is not more than half of No. 1.

### INDUSTRIAL APPLICABILITY

According to the present invention, it is possible to efficiently produce a steel pipe having a high roundness, without requiring excessive pressure.

### DESCRIPTION OF REFERENCE SYMBOLS

- 1: die
- 1a: rod-like member
- 1b: rod-like member
- 2: punch
- 2a: punch tip
- 2b: punch support
- 3: roller
- 4: upper die
- 4a: circular arc surface
- 4b: forming surface (inclined surface)
- 5: lower die
- 5a: circular arc surface
- S: plate material
- S₁: preformed body
- S₂: open pipe

## Claims

1. A method of producing a steel pipe in which a plate material (S) which is bent at width end portions is subjected to at least one bending along its widthwise direction to form a preformed body (S1) having a U-shaped cross-section, an open pipe (S2) with a gap portion in a longitudinal direction is formed by adding a bending force to the preformed body (S1) to press the preformed body (S1), and end surfaces of the gap portion of the open pipe (S2) are butt-joined to each other to form a steel pipe, the method comprising:
providing a lightly-bent portion to which a slighter curvature is applied as compared to other regions, or providing a non-bent portion (P) in which the bending is omitted in at least a part of the plate material (S) in performing the bending on the plate material (S); **characterized in**
**that** the bending force is applied to a part spaced apart from the center of the lightly-bent portion or the non-bent portion (P) by a distance within a range of W/4 ± 0.07W in a width end portion direction of the plate material, where W is the width of the plate material (S), without constraining the lightly-bent portion or the non-bent portion (P), in pressing the preformed body (S1) into the open pipe (S2), and
**that** the length (L) of the lightly-bent portion or the non-bent portion (P) along the widthwise direction of the plate material is not more than 10% of the plate material width (W).

2. The method of producing a steel pipe according to claim 1, **characterized in that** the center of the lightly-bent portion or the non-bent portion (P) is provided in a part spaced apart from the width end portion of the plate material (S) by an amount of W/4 ± 0.07W.

3. The method of producing a steel pipe according to claim 1 or 2, **characterized in that** two lightly-bent or non-bent portions are provided, one at each side of a widthwise center of the preformed body (S1) in the widthwise direction of the plate material (S) and that at the time of pressing of the preformed body (S1), the bending force is simultaneously applied to two parts each spaced apart from the center of the lightly-bent portion or the non-bent portion (P) toward the width end of the plate material (S) by an amount of W/4 ± 0.07W.

4. The method of producing a steel pipe according to any one of claims 1 to 3, **characterized in that** a press die (4, 5) is used to press the preformed body (S1) into the open pipe (S2), the preformed body (S1) is supported at its lowermost end in a U-shaped posture in which an opening portion of the preformed body (S1) is facing upward, when applying the bending force to press the preformed body (S1), the preformed body (S1) is supported at a part not on the line of action of the bending force, and when an opening angle of the preformed body (S1) is defined as θs and an angle of the bending force is defined as θf, the pressing of the preformed body (S1) is started under the condition of θf > θs, wherein a straight line (q) which symmetrically bisects the preformed body (S1) through the widthwise center is defined as a reference line, the opening angle (θs) of the preformed body (S1) is defined as an angle formed between the reference line (q) and a straight line (r) connecting the widthwise center (W/2) of the preformed body (S1) and the widthwise end portion of the preformed body (S1) and the angle (θf) of the bending force is determined by the press die shape and a friction coefficient of a press die surface, when an angle to the horizontal plane of a forming surface of the press die (4, 5) is defined as θd, and the friction coefficient of the press die surface is defined as µ, the angle θf is determined as θf = θd - tan⁻¹ (µ).

5. The method of producing a steel pipe according to claim 4, **characterized in that** at the time of pressing of the preformed body (S1), the forming surface of the press die (4, 5) does not come into contact with the lightly-bent portion or the non-bent portion (P).

6. The method of producing a steel pipe according to claim 4 or 5, **characterized in that** at the time of pressing of the preformed body, an axis of symmetry (O) of the press die used for pressing of the preformed body (S1) coincides with an axis of symmetry of the preformed body (S1).

7. The method of producing a steel pipe according to any one of claims 4 to 6, wherein the press die (4, 5) includes a pair of bending tools (4, 5) configured to interpose the preformed body (S1) with the U-shaped cross-section therebetween.

8. The method of producing a steel pipe according to claim 7, wherein at least one of the bending tools (4, 5) has a circular arc surface (4a, 5a) having a width center that lies on the axis of symmetry (O) of the press die (4, 5), and a forming surface having an inclined surface (4b) which leads to each of both ends of the circular arc surface (4a) and is directed toward the axis of symmetry (O) of the press die (4, 5).

## Patentansprüche

1. Verfahren zum Herstellen eines Stahlrohrs, bei dem ein Plattenmaterial (S), das an Breiten-Endabschnitten gebogen ist, wenigstens einem Biegen in seiner Breitenrichtung unterzogen wird, um einen vorgeformten Körper (S1) mit einem U-förmigen Querschnitt auszubilden, ein offenes Rohr (S2) mit einem Spaltabschnitt in einer Längsrichtung ausgebildet wird, indem eine Biegekraft auf den vorgeformten Körper (S1) ausgeübt wird, um den vorgeformten Körper (S1) zu pressen, und Endflächen des Spaltabschnitts des offenen Rohrs (S2) stumpf miteinander verbunden werden, um ein Stahlrohr auszubilden, wobei das Verfahren umfasst:
Bereitstellen eines leicht gebogenen Abschnitts, dem im Vergleich zu anderen Bereichen eine geringere Krümmung verliehen wird, oder Bereitstellen eines nicht gebogenen Abschnitts (P), in dem das Biegen in wenigstens einem Teil des Plattenmaterials (S) beim Durchführen des Biegens an dem Plattenmaterial (S) ausgelassen wird;
**dadurch gekennzeichnet, dass**
die Biegekraft beim Pressen des vorgeformten Körpers (S1) zu dem offenen Rohr (S2) auf einen Teil aufgebracht wird, der von der Mitte des leicht gebogenen Abschnitts oder
des nicht gebogenen Abschnitts (P) um eine Entfernung innerhalb eines Bereichs von W/4 ± 0,07W in einer Richtung eines Breiten-Endabschnitts des Plattenmaterials beabstandet ist, wobei W die Breite des Plattenmaterials (S) ist, ohne den leicht gebogenen Abschnitt oder den nicht gebogenen Abschnitt (P) einzuschränken, und
dass die Länge (L) des leicht gebogenen Abschnitts oder des nicht gebogenen Abschnitts (P) in der Breitenrichtung des Plattenmaterials nicht mehr als 10 % der Breite (W) des Plattenmaterials beträgt.

2. Verfahren zum Herstellen eines Stahlrohrs nach Anspruch 1, **dadurch gekennzeichnet, dass** sich die Mitte des leicht gebogenen Abschnitts oder des nicht gebogenen Abschnitts (P) in einem Teil befindet, der von dem Breiten-Endabschnitt des Plattenmaterials (S) um einen Betrag von W/4 ± 0,07 W beabstandet ist.

3. Verfahren zum Herstellen eines Stahlrohrs nach Anspruch 1 oder 2, **dadurch gekennzeichnet, dass** zwei leicht gebogene oder nicht gebogene Abschnitte vorhanden sind, das heißt ein Abschnitt an jeder Seite einer Breiten-Mitte des vorgeformten Körpers (S1) in der Breitenrichtung des Plattenmaterials (S), und dass zum Zeitpunkt des Pressens des vorgeformten Körpers (S1) die Biegekraft gleichzeitig auf zwei Teile aufgebracht wird, die jeweils von der Mitte des leicht gebogenen Abschnitts oder des nicht gebogenen Abschnitts (P) in Richtung des Breiten-Endes des Plattenmaterials (S) um einen Betrag von W/4 ± 0.07W beabstandet sind.

4. Verfahren zum Herstellen eines Stahlrohrs nach einem der Ansprüche 1 bis 3, **dadurch gekennzeichnet, dass** eine Pressform (4, 5) eingesetzt wird, um den vorgeformten Körper (S1) zu dem offenen Rohr (S2) zu pressen, wobei der vorgeformte Körper (S1) an seinem untersten Ende in einer U-förmigen Haltung getragen wird, in der ein Öffnungsabschnitt des vorgeformten Körpers (S1) nach oben gewandt ist, wenn die Biegekraft aufgebracht wird, um den vorgeformten Körper (S1) zu pressen, der vorgeformte Körper (S1) an einem Teil, der nicht auf der Wirkungslinie der Biegekraft liegt, getragen wird, und wenn ein Öffnungswinkel des vorgeformten Körpers (S1) als θs definiert ist und ein Winkel der Biegekraft als θf definiert ist, das Pressen des vorgeformten Körpers (S1) unter der Bedingung begonnen wird, dass θf > θs, wobei eine gerade Linie (q), die den vorgeformten Körper (S1) symmetrisch durch die Breiten-Mitte halbiert, als eine Bezugslinie definiert ist, der Öffnungswinkel (θs) des vorgeformten Körpers (S1) als ein Winkel definiert ist, der zwischen der Bezugslinie (q) und einer geraden Linie (r) gebildet wird, die die Breiten-Mitte (W/2) des vorgeformten Körpers (S1) und den Breiten-Endabschnitt des vorgeformten Körpers (S1) verbindet, und der Winkel (θf) der Biegekraft durch die Form der Pressform sowie einen Reibungskoeffizienten einer Oberfläche der Pressform bestimmt wird, wenn ein Winkel zu der horizontalen Ebene einer formenden Fläche der Pressform (4, 5) als θd definiert ist, und der Reibungskoeffizient der Oberfläche der Pressform als µ definiert ist, der Winkel θf als θf = θd - tan⁻¹ (µ) bestimmt wird.

5. Verfahren zum Herstellen eines Stahlrohrs nach Anspruch 4, **dadurch gekennzeichnet, dass** zum Zeitpunkt des Pressens des vorgeformten Körpers (S1) die formende Fläche der Pressform (4, 5) nicht mit dem leicht gebogenen Abschnitt oder dem nicht gebogenen Abschnitt (P) in Kontakt kommt.

6. Verfahren zum Herstellen eines Stahlrohrs nach Anspruch 4 oder 5, **dadurch gekennzeichnet, dass** zum Zeitpunkt des Pressens des vorgeformten Körpers eine Symmetrieachse (O) der zum Pressen des vorgeformten Körpers (S1) eingesetzten Pressform mit einer Symmetrieachse des vorgeformten Körpers (S1) zusammenfällt.

7. Verfahren zum Herstellen eines Stahlrohrs nach einem der Ansprüche 4 bis 6, wobei die Pressform (4, 5) ein Paar von Biegewerkzeugen (4, 5) einschließt, die so ausgeführt sind, dass der vorgeformte Körper (S1) mit dem U-förmigen Querschnitt zwischen ihnen angeordnet wird.

8. Verfahren zum Herstellen eines Stahlrohrs nach Anspruch 7, wobei wenigstens eines der Biegewerkzeuge (4, 5) eine Kreisbogenfläche (4a, 5a) mit einer Breiten-Mitte, die auf der Symmetrieachse (O) der Pressform (4, 5) liegt, sowie eine formende Fläche mit einer geneigten Fläche (4b) aufweist, die jeweils zu beiden Enden der Kreisbogenfläche (4a) führt und auf die Symmetrieachse (O) der Pressform (4, 5) zu gerichtet ist.

## Revendications

1. Procédé de production d'un tuyau en acier dans lequel un matériau en plaque (S) qui est courbé aux parties d'extrémité de largeur est soumis à au moins une courbure le long de sa direction de sens de largeur pour former un corps préformé (S1) présentant une section transversale en forme de U, un tuyau ouvert (S2) avec une partie d'écart dans une direction longitudinale est formé en ajoutant une force de courbure au corps préformé (S1) pour presser le corps préformé (S1), et des surfaces d'extrémité de la partie d'écart du tuyau ouvert (S2) sont jointes de bout à bout l'une à l'autre pour former un tuyau en acier, le procédé comprenant :
une fourniture d'une partie légèrement courbée à laquelle une courbure plus légère est appliquée comparée à d'autres zones, ou une fourniture d'une partie non courbée (P) dans laquelle la courbure est omise dans au moins une partie du matériau en plaque (S) en exécutant la courbure du matériau en plaque (S) ;
**caractérisé en ce que**
la force de courbure est appliquée à une partie éloignée par espacement du centre de la partie légèrement courbée ou de la partie non courbée (P) d'une distance au sein d'une plage de W/4 1 0,07 W dans une partie d'extrémité de largeur du matériau en plaque, où W est la largeur du matériau en plaque (S), sans contraindre la partie légèrement courbée ou la partie non courbée (P), en pressant le corps préformé (S1) dans le tuyau ouvert (S2), et
la longueur (L) de la partie légèrement courbée ou de la partie non courbée (P) le long de la direction de sens de largeur du matériau en plaque n'est pas supérieure à 10 % de la largeur de matériau en plaque (W).

2. Le procédé de production d'un tuyau d'acier selon la revendication 1, **caractérisé en ce que** le centre de la partie légèrement courbée ou de la partie non courbée (P) est disposé dans une partie éloignée par espacement de la partie d'extrémité de largeur du matériau en plaque (S) d'une quantité de W/4 1 0,07 W.

3. Le procédé de production d'un tuyau en acier selon la revendication 1 ou 2, **caractérisé en ce que** deux parties légèrement courbées ou non courbées (P) sont disposées, une sur chaque côté d'un centre de sens de largeur du corps préformé (S1) dans la direction de sens de largeur du matériau en plaque (S) et **en ce que** au moment d'une pression du corps préformé (S1), la force de courbure est simultanément appliquée à deux parties chacune éloignée par espacement du centre de la partie légèrement courbée ou de la partie non courbée (P) vers l'extrémité de largeur du matériau en plaque (S) d'une quantité de W/4 1 0,07 W.

4. Le procédé de production d'un tuyau en acier selon l'une quelconque des revendications 1 à 3, **caractérisé en ce que** une matrice de presse (4, 5) est utilisée pour presser le corps préformé (S1) dans le tuyau ouvert (S2), le corps préformé (S1) est soutenu à son extrémité la plus basse dans une position en forme de U dans laquelle une partie d'ouverture du corps préformé (S1) est orientée vers le haut, lors d'une application de la force de courbure pour presser le corps préformé (S1), le corps préformé (S1) est soutenu sur une partie hors de la ligne d'application de la force de courbure, et lorsqu'un angle d'ouverture du corps préformé (S1) est défini comme θs et un angle de la force de courbure est défini comme θf, la pression du corps préformé (S1) est initiée sous la condition de θf > θs, dans lequel une ligne droite (q) qui coupe symétriquement le corps préformé (S1) via le centre de sens de largeur est définie en tant que ligne de référence, l'angle d'ouverture (θs) du corps préformé (S1) est défini en tant qu'angle formé entre la ligne de référence (q) et une ligne droite (r) connectant le centre de sens de largeur (W/2) du corps préformé (S1) et la partie d'extrémité de sens de largeur du corps préformé (S1) et l'angle (θf) de la force de courbure est déterminé par la forme de la matrice de presse et un coefficient de friction d'une surface de matrice de presse, lorsqu'un angle au plan horizontal d'une surface de formation de la matrice de presse (4, 5) est défini comme θd, et le coefficient de friction de la surface de matrice de presse est défini comme µ, l'angle de θf est déterminé comme θf = θd - tan⁻¹ (µ).

5. Le procédé de production d'un tuyau en acier selon la revendication 4, **caractérisé en ce que** au moment de pression du corps préformé (S1), la surface de formation de la matrice de presse (4, 5) n'entre pas en contact avec la partie légèrement courbée ou la partie non courbée (P).

6. Le procédé de production d'un tuyau en acier selon la revendication 4 ou 5, **caractérisé en ce que** au moment de pression du corps préformé, un axe de symétrie (O) de la matrice de presse utilisée pour presser le corps préformé (S1) coïncide avec un axe de symétrie du corps préformé (S1).

7. Le procédé de production d'un tuyau en acier selon l'une quelconque des revendications 4 à 6, dans lequel la matrice de presse (4, 5) inclut une paire d'outils de courbure (4, 5) configurés pour interposer le corps préformé (S1) avec une section transversale en forme de U entre ceux-ci.

8. Le procédé de production d'un tuyau en acier selon la revendication 7, dans lequel au moins un des outils de courbure (4, 5) présente une surface en arc circulaire (4a, 5a) présentant un centre de largeur qui se trouve sur l'axe de symétrie (O) de la matrice de presse (4, 5), et une surface de formation présentant une surface inclinée (4b) qui conduit aux deux extrémités de la surface en arc circulaire (4a) et est dirigée vers l'axe de symétrie (O) de la matrice de presse (4, 5).
